

## UNITED STATES PATENT OFFICE

2,257,088

## WATER-REPELLENT PROCESS

Herman A. Bruson and Louis H. Bock, Philadelphia, Pa., assignors to Röhm & Haas Company, Philadelphia, Pa.

No Drawing. Application December 29, 1938,  
Serial No. 248,196

7 Claims. (Cl. 8—113)

This invention relates to a new process of rendering textile fabrics, yarns, and fibers water-repellent without materially altering the general appearance of the fabric.

Water-repellency is obtained by imparting to the surface of fibers a waxy finish which is not easily wet by water. In the usual process of waterproofing fabrics the surface of the fabric is coated with a superficial layer of a wax or a metallic soap. These water-repelling substances are relatively easily removed by solvents in dry cleaning baths or by hot soap solutions in laundering. Recently various chemical treatments of cellulose fibers have been suggested, but thus far these methods have suffered from certain disadvantages, such as resulting loss of tensile strength or evolution of unpleasant or toxic fumes during the processing of the fabric.

The object of this invention is to provide a process of imparting to fibers, yarns, and fabrics a highly water-repellent finish which is permanent to laundering and dry cleaning. Another object is to impart the property of water-repellency to all the fibers within the fabric and avoid superficial coating of fabric. A further object is to provide permanent water-repellency with retention of the strength of the fabric. A further object is to provide water-repelling agents which do not evolve toxic fumes during processing.

It has been found that these objects may be attained by the use of compounds possessing the following general structure—



in which Ar represents an aromatic nucleus of the benzene or naphthalene series carrying a nuclearly bound oxygen atom and at least one hydrocarbon substituent of the aliphatic or cycloaliphatic series which contains eight or more carbon atoms and which is bound to the aromatic nucleus directly or through an ether, carbonyl, carboxyl or carbamido linkage. The nuclearly bound oxygen may be part of a hydroxyl group or part of a side chain. In the above formula A and B represents members of the group consisting of open chain, lower aliphatic groups when taken singly and when taken together divalent groups which jointly with the nitrogen form a heterocycle.

The hydrocarbon substituents may be such groups as primary, secondary, or tertiary octyl, dodecyl, hexadecyl or octadecyl groups, unsaturated groups such as undecenyl or octadecenyl,

alicyclic groups such as bornyl, camphyl, naphthenyl or butyl cyclohexyl. More than one such group may be present.

The compounds may be obtained by condensing a phenolic derivative containing an aliphatic or cycloaliphatic side chain of at least eight carbon atoms with formaldehyde and a non-aromatic secondary amine. In another modification a suitable phenol is condensed with formaldehyde and a non-aromatic secondary amine and the hydroxyl group is esterified with an acyl halide containing more than seven carbon atoms or the hydroxyl group may be etherified with a long chain hydrocarbon group.

These compounds may be used in the form of the free base or in the form of a salt obtained by neutralizing the base with an organic or inorganic acid or by reacting with an agent for alkylation to yield a quaternary ammonium salt. Compounds possessing the essential groups and linkages have been described in U. S. patents to Bruson Nos. 2,033,092; 2,040,039 and 2,040,040 and in U. S. Serial No. 240,009 filed November 12, 1938, now Patent No. 2,218,739, and in U. S. Serial No. 244,923 filed December 1, 1938.

The quaternary ammonium salts are usually the preferred form for use since they may be used directly in aqueous baths with or without a catalyst. The catalyst may be acidic or basic as desired. But, as shown above, either the base or the salt forms may be used by being taken up in water or other solvent for application to fabrics or yarns. Dispersions or solutions are quite stable.

Products of the general type described have the advantages of being well dispersed or dissolved by water and being soap-like in properties, providing wetting and penetrating actions. They are adsorbed by the fibers and when the fabric is subsequently heated, these compounds react with the fibers to form water-repellent derivatives of the fibers themselves. The wetting and penetrating actions are particularly important because, as a result of penetration, the fibers throughout a fabric and not merely the surface of the fabric become water-repellent.

Since these compounds are soap-like, they form solutions which may contain ions and molecules, and also micelles or molecular aggregates. The term "solution" as used for such substances includes the usual sort of solution and the dispersions of the molecular aggregates.

While it may appear surprising at first glance that a soap-like compound which possesses wetting, penetrating and emulsifying properties

should become a good water-repellent, the behavior is readily explained. All capillary-active compounds contain within their molecules polar and non-polar groupings. Ordinarily, it is not easy to separate these two parts of the molecule. The applicants have found, however, that certain compounds which possess the aryl methylene nitrogen-linkage are decomposed, when heated on fibers, with the formation of a compound of the fiber itself with the non-polar part of the soap-like molecule. In the case of cellulose, a cellulose ether is believed to be formed. The resulting compound is hydrophobic and stable, and cannot be removed without serious damage to the fiber.

The aryl-methylene amines and their salts are effective not only on cellulose fibers such as cotton, rayon, straw, kapok, and linen, but also on wool and silk. Any of the usual organic materials which are used for making yarns, sheets, fabrics, battings, etc., and which are not damaged by heating to 120° C. or more may be treated by the herein disclosed process.

The process of treating fabric, yarn, or even loose fiber is relatively simple. The material to be treated is impregnated with the solution by any convenient method, such as padding, dipping, spraying, etc. Then, with or without previous drying, the material is subjected to a temperature high enough to bring about the reaction of the compound and the fiber. The preferred temperature for this reaction is above about 120° C. The time required for the reaction will vary with the temperature used. At 120° C., for example, an hour may be required, whereas two or three minutes is usually sufficient at 150° C. It is desirable to remove the by-products of the reaction by washing the textile material after it has been heated.

Solutions containing the tertiary salts and also solutions containing the quaternary salts are usually acid. The excess acid seems to serve as a catalyst in promoting the reaction between the compound and the fibers, although a catalyst is not essential to the process. On the other hand, it has been found that alkaline salts such as sodium carbonate or sodium acetate are also useful catalysts in the reaction.

Not all the aryl-methylene nitrogen compounds are soluble in mildly alkaline solutions. Those compounds, however, containing a free hydroxyl group tend to be soluble. Compounds derived from acyl phenols are usually sufficiently soluble in slightly alkaline solutions to permit their use in this way. There is practically no danger of tendering fabric with such solutions.

The following examples are given to illustrate the method of rendering fibers water-repellent but they are not to be interpreted as limitations thereof.

*Example 1.*—Cotton broadcloth was immersed in a solution containing 5 parts of acetic acid, 87 parts of water and 8 parts of the condensation product of equimolecular quantities of octadecyl phenol, formaldehyde and dimethylamine having the formula—



The cloth was dried at room temperature and baked 30 minutes at 130° C. It was very water-repellent and it retained this property after repeated washing in hot soap solution.

*Example 2.*—Cotton sheeting was immersed in a solution containing 5 parts of acetic acid, 90

parts of water and 5 parts of the condensation product of octadecyl phenol, formaldehyde and morpholine having the formula—



The fabric was squeezed as dry as possible and pressed with a hot flat iron for 3 minutes. A wash-fast, water-repellent finish resulted.

Example 3.—Viscose rayon was treated with a solution containing 8 parts of hexadecyl-hydroxybenzyl-diethylamine (obtained by the condensation of hexadecyl phenol with formaldehyde and diethylamine), 5 parts of formic acid, and 87 parts of water. The material was dried in an oven at 130° C. for one hour. Good water-repellency was obtained.

20 *Example 4.*—Wool fabric was wet out in a solution containing 10 parts of the oleic acid ester of hydroxybenzyl dimethyl benzyl ammonium chloride in 90 parts of water. The fabric was dried at room temperature and baked in a closed oven 30 minutes at 130° C. The finished material had excellent water-repellency which resisted a hot soap wash.

Example 5.—Cotton sheeting was immersed in a solution containing 5 parts of acetic acid, 87 parts of water and 8 parts of the  $\beta$ -chloroethoxy ethyl ether of the condensation product of p-( $\alpha$ ,  $\alpha$ ,  $\gamma$ ,  $\gamma$ -tetramethylbutyl) phenol, formaldehyde and dimethylamine. The fabric was placed in an oven at 150° C. for 10 minutes. After washing, the material retained a considerable degree of water-repellency.

Example 6.—Cotton yarn was immersed in a solution containing 10 parts of the lauric ester of hydroxyl benzyl dimethyl benzyl ammonium chloride and 90 parts of water. After drying at room temperature, it was heated 10 minutes at 140° C. A good, permanent, water-repellent finish was obtained.

*Example 7.*—Cotton sheeting was immersed in a solution containing 10 parts of the condensation product of stearoyl phenol, formaldehyde and dimethylamine, 1 part of sodium carbonate, and 89 parts of water. It was baked 30 minutes at 125° C. Permanent water-repellency resulted.

50      *Example 8.*—Cotton toweling was immersed in  
a solution containing 10 parts of the naphthenic  
ester of hydroxybenzyl dimethyl benzyl ammonium  
chloride and 90 parts of water. It was baked  
55      30 minutes at 130° C. The cotton was very wa-  
ter-repellent after washing in hot soap solution.

Example 9.—Cotton sheeting was immersed in a solution containing 10 parts of p-stearamido-hydroxy benzyl-dimethylamine and 100 parts of water containing 5 g. of acetic acid. After drying at room temperature it was heated 10 minutes at 135° C. A good water-repellent finish was obtained. The stearamido hydroxybenzyl dimethylamine was obtained by heating equimolecular quantities of p-stearamidophenol, formaldehyde and dimethylamine in alcohol solution for 2 hours.

70 While agents of the sort described herein may be applied in organic solvents, treatment of fabric with the agents in water avoids the hazards of applying such agents in solvents which are apt to be inflammable or toxic. In this invention the use of soap-like materials not only provides wetting and penetrating actions but also 75 emulsifying action, which permits the incorpora-

tion of small amounts of waxes or other inexpensive waterproofing agents in the treating bath. While such waxes are not permanent, like the reaction product of the aryl-methylene amines with fibers, they aid initial repellency at a minimum of expense. Whether the new water-repellent agents are used alone or in combination with other water-repellent materials, they offer the advantage of a one-bath process.

We claim:

1. The process of treating textile material, which comprises impregnating the material with a compound selected from the group consisting of phenolic-methylene tertiary amines in which two of the N-substituents are chosen from the group consisting of open chain, lower aliphatic groups and divalent groups which jointly with the nitrogen form a heterocyclic ring and in which the phenolic group bears an organic substituent of the aliphatic and cycloaliphatic series containing at least eight carbon atoms, the acid salts of said amines, and the quaternary salts of said amines, and subsequently heating said textile material to react the amine compound therewith.

2. The process of treating textile material, which comprises impregnating the material with a bath containing a benzyl amine in which two of the N-substituents are lower aliphatic groups and in which the phenyl group carries nuclearly bound oxygen and a hydrocarbon substituent of at least eight carbon atoms obtainable from the aliphatic and alicyclic series, and subsequently heating said textile material to react the benzyl amine therewith.

3. The process of treating textile material, which comprises impregnating the textile material with an alkaline aqueous dispersion of octadecyl hydroxy benzyl dimethylamine, and

subsequently heating said textile material to react the benzyl dimethylamine therewith.

4. The process of treating textile material, which comprises impregnating the material with an aqueous solution of an acid salt of a benzyl amine in which two of the N-substituents are lower aliphatic groups and in which the phenyl group carries nuclearly-bound oxygen atom and a hydrocarbon substituent of at least eight carbon atoms obtainable from the aliphatic and alicyclic series, and subsequently heating said textile material to react the benzyl amine therewith.

5. The process of treating textile material, which comprises impregnating the textile material with an aqueous solution of the acetic acid salt of octadecyl hydroxy benzyl dimethylamine, and subsequently heating said textile material to react the benzyl dimethylamine therewith.

6. The process of treating textile material, which comprises impregnating the material with an aqueous solution of a quaternary salt of a benzyl amine in which at least two of the N-substituents are lower aliphatic groups and in which the phenyl group contains a substituent of at least eight carbon atoms obtainable from the aliphatic and alicyclic series joined to the phenyl group by a carboxyl linkage, and subsequently heating said textile material to react the benzyl amine therewith.

7. The process of treating textile material, which comprises impregnating the material with an aqueous solution of the oleic acid ester of hydroxyl benzyl dimethyl benzyl ammonium chloride, and subsequently heating said textile fabric to react the quaternary ammonium salt therewith.

HERMAN A. BRUSON.  
LOUIS H. BOCK.